

## UNITED STATES PATENT OFFICE

2,494,765

## CHEMICAL ERASING OF PHOTOGRAPHIC SILVER IMAGES

John F. Kienast, River Edge, N. J., assignor to  
Keuffel & Esser Company, Hoboken, N. J., a  
corporation of New Jersey

No Drawing. Application November 10, 1944,  
Serial No. 562,916

7 Claims. (Cl. 95—88)

1

This invention relates to a method for and compositions useful in the making of erasures on photographic prints.

In engineering reproduction materials and particularly those which employ silver to produce the visible image, it is oftentimes desirable to make erasures by removing the silver which colors some of the areas, either to correct errors or to remove lines from certain portions in order that they may be corrected or redrawn.

The invention is applicable to many types of photographic materials on various base stocks such as paper, cloth, film, sheet metal, etc., including: those commonly referred to as vandykes, brown prints and the like where the image is created from a combined soluble silver salt and an iron salt; engineering reproduction materials with silver halide emulsions; engineering reproduction materials having gum or glue bichromate with silver images and the like; and may also be used for correcting ordinary photographic film as well as photographic prints which latter are oftentimes referred to as photoprints or photocopies.

In the past, various procedures have been proposed for making the corrections in a silver image and one of the early methods included the application of a single fluid eradicator, the principal constituent of which was mercuric chloride. Erasures made with this material were fugitive and became opaque when exposed to light, corroded pens and drawing instruments which were later used on the areas, had some danger from toxicity and produced "ghosts" which showed up when the photographic material was used for reproduction purposes.

Some improvement in erasing fluids occurred by applying hypochlorite in the form of sodium hypochlorite which was the first step in removing the image. For the second step the area was treated with a hypo fixing solution. Results were not generally satisfactory or uniform because it was difficult to stabilize the hypochlorite which deteriorated in storage or, if stabilized with alkali, had a deleterious effect on the base material when applied to make an erasure. It was difficult to make a drawing over an erased area particularly when ink lines were employed, as the ink spread through the base which was often so weakened that it would crack or disintegrate.

It has now been discovered that the undesirable effects and disadvantages of prior art methods can be avoided by using two solutions successively in the manner hereinafter described, when it is

2

desired to make erasures of images which were created photographically from silver salts.

In order to carry out this invention, a cupric halide, preferably cupric chloride, is dissolved in water in quantities ranging from 3% to 50% with best results obtained from cupric chloride representing approximately 15%. This material is stable in storage, the desired concentration is readily secured and it does not in any manner

10 attack the base sheet.

Improved results are obtained by the addition of an ammonium halide which may correspond with the cupric salt. Where this is ammonium chloride, it is used in amounts ranging from a 15 concentration of 5% to as high as 25% with amounts approximately 15% being satisfactory for most purposes. The solubility of the ammonium chloride is determined by the amount of the cupric chloride already in solution, that is, 20 the greater the concentration of cupric chloride the less ammonium chloride will go into solution. It is preferable to use the maximum quantity that can be dissolved in the cupric chloride solution already prepared. The ammonium chloride 25 improves the action of the first fluid by increasing the speed of the first reaction and it also makes possible a final erasure after the second fluid is applied, which is somewhat cleaner, i. e. more complete, than if the cupric chloride is used 30 alone in the first solution.

A preferred solution has the following proportions:

Distilled water, 1000 cc.  
Cupric chloride ( $CuCl_2 \cdot 2H_2O$ ), 167 gms.  
Ammonium chloride, 167 gms.  
10% di hexyl sodium sulfosuccinate solution, 8 cc.

35 The second solution used for making erasures is an aqueous solution of thiourea. Preferably, this solution also contains a suitable wetting agent of the types herein set forth. In the preferred composition the thiourea is dissolved in water to make a saturated solution. About one and one-quarter ( $1\frac{1}{4}$  lbs.) pounds will dissolve in one gallon of water at normal room temperatures. Such a solution with small amounts of a wetting agent is stable under conditions of normal storage and use.

40 To either the erasing fluid or the fixing fluid or both, a wetting agent such as alcohol, sulphonated alcohol, di hexyl sodium sulfosuccinate or the like may be added in small amounts.

45 In order to make an erasure, the cupric chloride solution, with or without ammonium chloride and a wetting agent, is applied to the area where the

erasure is desired, with a brush, cloth, glass applicator or the like and rubbed into the surface. Preferably the rubbing is continued until the image has disappeared although this is not necessary and the cupric chloride solution may be blotted from the surface promptly after it has been applied uniformly over the area to be treated. After the excess liquid has been removed by blotting, the second solution of thiourea and the wetting agent is applied to the same area though for many types of engineering reproductions it need not be so limited. The solution may be permitted to dry on the sheet but it is usually preferred to remove the residual liquid as by blotting. It can, of course, be washed from the surface in any known manner but this results in unduly wetting the sheet and is preferably avoided.

The combination of the cupric chloride solution and the thiourea solution for erasing has many advantages over other erasing fluids. A prior two-fluid combination for erasing which included a first solution comprising cupric chloride presented difficulties in use because it was necessary to insure thorough conversion of the image with the cupric chloride before its blotting and the application of a fixing solution, otherwise the erasure will not be complete and even if the process is carried out carefully it is possible that there may be some staining of the print, a condition which is particularly undesirable where engineering reproductions are concerned. This was likely to occur in those cases where the print had been prepared under conditions where special treatments had been given either to accelerate the original reproduction process or where final washing was inadequate or incomplete. Under such cases residual salts left in the base material adversely affected the erasing action and in some instances resulted in producing colored compounds that left an apparently permanent stain in the drawing.

Where the present composition is used, i. e. the thiourea solution is applied to the print after treatment with the cupric chloride solution, the critical procedural details formerly necessary can be dispensed with. Excellent erasures are secured even where residual salts from the original development have not been adequately or completely removed. The erasure restores the original color of the base sheet.

Instead of using cupric chloride for the first solution, other oxidizing or decolorizing solutions may be employed. Another is ammonium or potassium persulfate saturated solution which, however, has no discernable effect when first applied but produces the erasure when the solution of thiourea is also present. These two solutions cannot be premixed though both must be present simultaneously.

The compositions herein described, when used in the process as set forth, will remove silver images from paper, cloth, film, metal or other bases normally used as supports for light-sensitive layers containing silver and will produce erasures which are very permanent and do not affect the base either as to strength or as to ability to receive redrawn lines. The erasure does not leave any residue which appears on the print when the erased sheet is used in making reproductions as, for example, by contact printing.

The cupric chloride required in the first fluid may be obtained not only by dissolving the salt cupric chloride in water but also by providing

in solution the divalent cupric ion from any other source such as copper sulfate and the chloride ion from any suitable chloride salt as, for example, sodium chloride thereby providing in the solution the divalent cupric ion and the chloride ion. The ammonium chloride desired in the solution may also be provided by the ionization of ammonium salts and chloride salts.

Other cupric halides in addition to the cupric chloride discussed above may be used although results are generally not as effective. For example, cupric bromide works very slowly and the addition of ammonium bromide has no noticeable effect. On the other hand, the addition of ammonium chloride greatly improves the action. Cupric fluoride works slowly upon the addition of ammonium fluoride and, of course, more rapidly if ammonium chloride is added.

It should be understood that where reference is made to a solution of cupric halide, this expression is intended to mean that the solution contains cupric ions and halide ions even though not obtained directly by the solution of the cupric halide.

While the invention has been described with reference to certain preferred procedures and compositions, these are to be considered as illustrative of the invention as defined in the appended claims.

I claim:

1. The process for erasing silver images on bases which comprises applying to that portion of the image which is to be erased a solution containing between 3 and 50% of cupric chloride and from 25 to 5% of ammonium chloride, treating the area to which the cupric chloride solution was applied with a substantially saturated solution of thiourea and removing the resulting solution.

2. The process for erasing silver images on bases which comprises applying to that portion of the image which is to be erased a solution containing 15% cupric chloride and 15% ammonium chloride, treating the area to which the cupric chloride solution was applied with a substantially saturated solution of thiourea and removing the resulting solution.

3. A composition for making erasures of silver images which comprises an aqueous solution consisting essentially of 3 to 50% cupric chloride and ammonium chloride in a sufficient concentration of from 25 to 5% to form a substantially saturated solution in water.

4. A composition for making erasures of silver images which comprises an aqueous solution consisting essentially of a wetting agent, from 3 to 50% cupric chloride and ammonium chloride in a sufficient concentration of from 25 to 5% to form a substantially saturated solution in water.

5. A composition for making erasures of silver images by applying the composition to that portion of the image which is to be erased and thereafter treating the area to which the composition has been applied with a substantially saturated solution of thiourea, said composition consisting essentially of approximately 15% cupric chloride and ammonium chloride in a sufficient concentration of approximately 15% to form a substantially saturated solution in water.

6. The process for erasing silver images on bases which comprises applying to that portion of the image which is to be erased a solution containing between 3 and 50% of cupric chloride, treating the area to which the cupric chlo-

ride solution was applied with a substantially saturated solution of thiourea and removing the resulting solution.

7. A composition for making erasures of silver images by applying the composition to that portion of the image which is to be erased and thereafter treating the area to which the composition has been applied with a substantially saturated solution of thiourea, said composition consisting essentially of 3 to 50% cupric chloride and ammonium chloride in a sufficient concentration of from 25 to 5% to form a substantially saturated solution in water.

JOHN F. KIENAST.

REFERENCES CITED

The following references are of record in the file of this patent:

UNITED STATES PATENTS

| Number    | Name           | Date          |
|-----------|----------------|---------------|
| 1,780,025 | Mankenberg     | Oct. 28, 1930 |
| 1,945,658 | Roessler       | Feb. 6, 1934  |
| 1,963,197 | Frohlich       | June 19, 1934 |
| 2,000,353 | Schaeffer      | May 7, 1935   |
| 2,100,594 | Heymer         | Nov. 30, 1937 |
| 2,107,094 | Townsend       | Feb. 1, 1938  |
| 2,166,617 | Weber et al.   | July 18, 1939 |
| 2,311,015 | Young et al.   | Feb. 16, 1943 |
| 2,322,084 | Young et al.   | June 15, 1943 |
| 2,327,822 | Russell et al. | Aug. 24, 1943 |

OTHER REFERENCES

- 16 Clerc: "Photography Theory and Practice," Pitman & Sons, New York, 1937, p. 270 cited.